

Nov. 22, 1949

M. M. STRIPLIN, JR., ET AL

2,488,568

PRODUCTION OF ALUMINUM-SILICON ALLOYS

Filed May 20, 1948

2 Sheets-Sheet 1



FIG. 1



FIG. 2

Marcus M. Striplin Jr. and <sup>INVENTORS</sup>  
William M. Kelley  
BY Bentley C. Morrow  
Attorney

Nov. 22, 1949

M. M. STRIPLIN, JR., ET AL

2,488,568

PRODUCTION OF ALUMINUM-SILICON ALLOYS

Filed May 20, 1948

2 Sheets-Sheet 2



FIG. 3

Marcus M. Striplin Jr. and INVENTOR.  
William M. Kelley  
BY Bentley O'Morrow  
Attorney

## UNITED STATES PATENT OFFICE

2,488,568

## PRODUCTION OF ALUMINUM-SILICON ALLOYS

Marcus M. Striplin, Jr., Florence, Ala., and William M. Kelly, Niagara Falls, N. Y., assignors to Tennessee Valley Authority, a corporation of the United States

Application May 20, 1948, Serial No. 28,266

12 Claims. (Cl. 75—10)

(Granted under the act of March 3, 1883, as amended April 30, 1928; 370 O. G. 757)

1

The invention herein described may be manufactured and used by or for the Government for governmental purposes without the payment to us of any royalty therefor.

This invention relates to improved methods for the manufacture of aluminum-silicon alloys by reducing oxides or ores of aluminum and silicon with carbon in electric furnaces. It relates particularly to means for reducing power and electrode consumption in the process.

It has long been known that aluminum-silicon alloys may be produced by heating clay or mixtures of clay with such materials as bauxite or silica pebble or sand with sufficient carbon as reducing agent, preferably in the form of coke or charcoal, to reduce the charge to an alloy of aluminum, silicon and the other metallic constituents which may be present, usually iron or titanium. Oxides of aluminum and silicon from whatever source obtained might be used in this process, but the cheapness and wide availability of clay makes clay the more common starting material to be used.

The process is usually carried out in an electric furnace because of the high temperature required for reduction, which is of the order of about 2000° C. Heat is produced by the resistance of the charge to the flow of current and by arcing. When the required temperature is reached, reduction begins and the reduced metals collect in a pool in the bottom of the furnace from whence the resulting alloy is tapped out periodically.

Aluminum-silicon alloys are useful as reducing agents in the deoxidation of steel. They have also been used as a source of aluminum and silicon in the manufacture of "Silumin," an aluminum-silicon casting alloy containing about 12 per cent silicon. They have been found to have advantages over ferrosilicon as a reducing agent in the production of magnesium from dolomite. In addition to these applications, there is a possibility of obtaining relatively pure aluminum and silicon from the alloys. A method of the latter type is shown in the U. S. Patent 2,469,418.

Production of aluminum-silicon alloys is in many respects similar to production of ferroalloys, such as ferrosilicon. The same types of furnaces are used and most of the operating conditions are similar. One of the differences is in the amount of electrode carbon consumed in the reduction. For example, in ferrosilicon manufacture, carbon electrode consumption ranges from 110 to 130 pounds per ton of product when a charge contains approximately the amount of carbon stoichiometrically required to reduce the oxides in the charge to their elements with the formation of an equivalent

2

amount of carbon monoxide. In contrast, operation of an aluminum-silicon alloy process in an electric furnace with a charge containing coke in corresponding proportions will result in a carbon electrode consumption of more than 500 pounds per ton of alloy. And, in addition, conditions will develop in the furnace which cause a shut-down in relatively short time. This high electrode consumption and difficulty in getting continuous furnace operation have been the main disadvantages in the prior art processes for the manufacture of aluminum-silicon alloys.

It is common practice in the production of ferroalloys to use close to or, in some cases, slightly more than the amount of carbon theoretically necessary to reduce all the metal oxides present, as is shown in *Electrochemistry*, by W. A. Koehler, John Wiley and Sons, New York (1935), page 414. This practice has also been followed in the manufacture of aluminum-silicon alloys, as is shown by British Patent No. 302,692, December 20, 1927. Attempts have been made to reduce electrode consumption by increasing the proportion of carbon in the charge since it is logical to assume that oxidation of the carbon on the electrodes results from attack by the oxides in the charge and that this can be reduced by the provision of additional carbon in the charge. In the somewhat similar process of reducing phosphate rock to form elemental phosphorus in electric furnaces, such procedure has been very effective, as is shown by R. H. Newton in *Chemical and Metallurgical Engineering*, 45, page 536-540, (1938). Increase in the carbon content of the charge from 100 per cent to 103 per cent and 106 per cent has decreased the electrode consumption from 34 to 29 and 11 pounds per ton of P<sub>2</sub>O<sub>5</sub> charged, respectively. However, when increase of carbon content in the charge in the preparation of an aluminum-silicon alloy is attempted, no decrease in electrode consumption follows.

It is an object of this invention to provide an improved process for the production of an aluminum-silicon alloy in an electric furnace.

Another object is to provide a novel and beneficial ratio of carbon to oxides in the charge used in such a process.

Another object is to provide advantageous electrical operating conditions adapted to be used in connection with such novel and advantageous ratio of carbon to oxide to secure lowered electrode consumption and lower power consumption per ton of alloy produced.

Still another object is to provide an improved process for the production of an aluminum-silicon alloy which is characterized by lowered electrode consumption.

Other objects and advantages will become apparent as this disclosure proceeds.

We have now found that electrode consumption per ton of alloy produced can be materially decreased and furnace operation improved in the aluminum-silicon alloy process by restricting the amount of carbon used as reducing agent to an amount not greater than 85 per cent of the stoichiometrical amount required to reduce the total oxides in the charge to their elements and form an equivalent amount of carbon monoxide. It is advantageous in our process to use from 67 to 85 per cent of the amount of carbon theoretically required for reducing the oxides present and for most types of charge there is a particularly advantageous range which is from 70 to 75 per cent of such theoretical amount. The electrode consumption per ton of product drops off sharply with decrease in the proportion of reducing agent from about 85 per cent until a minimum is reached, in the neighborhood of 70 to 75 per cent and steady state furnace operation becomes possible. If the ratio is decreased further, the trend is reversed and there is some increase in electrode consumption.

We have also found that there are certain electrical conditions which may be used in combination with my novel ratio of carbon to oxides in the charge to give maximum decrease in electrode consumption and to give a substantial decrease in power required per ton of alloy produced. These electrical conditions are not effective unless used in combination with our novel ratio of carbon to oxides in the charge.

These electrical conditions may be conveniently expressed in terms of a factor R, which is defined as follows:

$$R = \frac{E}{I} \times \pi \times D$$

where E equals the potential drop from electrode to hearth measured in volts, I equals current per electrode in amperes and D equals electrode diameter in inches. This factor is seen to have the dimensions of ohm-inches and is, in effect, the resistance per inch of electrode circumference if the path of the circuit from the electrode to the hearth is considered as consisting of parallel circuits, the number depending on the electrode circumference. This factor R is hereinafter in this disclosure and claims referred to as electrode periphery resistance R and is measured in ohm-inches.

We have found that there is a certain critical range for R which, when combined with use of the proper proportions of carbon, gives a relatively low consumption of electrode. Increase or decrease of R from the critical range even with the optimum amount of reducing agent gives some increase in electrode consumption. On the other hand, use of the proper value of R is of no advantage if the proportion of reducing agent, i. e. carbon, in the charge is too high. Steady state operation of the furnace becomes impossible and electrode consumption is high at any value of R. In the attached drawing, Figure 1 is a graph in which the lower curve A shows the decrease in electrode consumption in relationship to decrease in carbon content of charge. The upper curve B in the same figure shows decrease in power consumption per pound of alloy with decrease of carbon content of charge. Figure 2 is a graph in which curve A shows decrease in electrode consumption with increase in electrode periphery resistance R in ohm-inches when the

carbon in the charge is maintained constant at about 70 per cent of the theoretical. Curve B in this graph shows decrease in power consumption under the same conditions. These curves were obtained by the use of a charge composed essentially of clay in admixture with coke and were obtained by the use of a graphite electrode. Curves of similar shape but differing in the point of minimum were obtained with charges of different composition and with the electrodes of other forms of carbon. It will be seen that greatest efficiency is shown when R is between the values of 0.14 and 0.16 when graphite electrodes are used. When electrodes formed from amorphous carbon are used, this figure for R is changed and the greatest efficiency is obtained when the values of R lie between 0.30 and 0.45, with 0.33 being the usual minimum. This is shown by Figure 3, a graph similar to Figure 2, but obtained by the use of electrodes formed from amorphous carbon. Partially graphitized electrodes give curves having optimum values between those shown in Figure 2 and Figure 3. Thus it will be seen that the optimum value for R varies with the type of carbon used in the electrodes, but will lie in the range from 0.14 to 0.45.

Since, because of its cheapness, clay is the favored material for producing such alloys, these graphs are confined to the use of clay. It is possible, however, to increase the proportion of aluminum by the addition of a high-alumina raw material such as bauxite to the furnace charge or to increase the proportion of silica by the addition of silica rock. Such variations in the charge require certain variations in the carbon content in order to give the greatest efficiency and the greatest decrease in electrode consumption. Such charges, however, give curves very similar in shape to those shown in the attached graph, although the minimum shown in relationship to the carbon content of the charge may vary considerably from that shown. For instance, when a charge of clay and silica rock in such proportions as to produce an alloy containing approximately 75 per cent silicon is used, we have found that the minimum electrode consumption was obtained when the charge contained 81 per cent of the coke theoretically required for reduction of all oxides present. Since there are a great number of such variations in the charge possible, each having a slightly different point of minimum electrode consumption, it is impractical to show all such possible variations. However, these may be easily determined by methods well-known to the art by selecting ratios between 67 and 85 per cent of the carbon theoretically required and plotting a graph similar to that illustrated.

The ratio of carbon to total oxides must be not greater than the minimum ratio at which the resulting alloy is substantially free from infusible material and must exceed the maximum quantity at which a substantial proportion of slag is formed.

The optimum proportion of carbon present in the charge as reducing agent is not affected by the type of carbon electrodes used. Thus when optimum results are given by a clay charge containing from 70 to 75 per cent of the carbon theoretically required for reducing the total metal oxides present when a graphite electrode is used, no change in optimum proportions occurs when electrodes formed from amorphous carbon are substituted for graphite ones.

The electrode periphery resistance R may be varied by raising or lowering the position of elec-

trodes in the furnace, by changing the size or diameter of electrodes or by varying the voltage applied to the electrodes. All these methods are well-known in the art and will not be described fully. No particular type of electric furnace is necessary for carrying out our novel process. Almost any arc-resistance electric furnace well-known in the art may be used. No particular machinery or equipment for preparing the charge is a part of our invention, which is confined to a process for preparing aluminum-silicon alloys. Details and advantages of our process will become apparent from consideration of the following examples. Example I illustrates the disadvantages which follow from the use of the methods of the prior art and Examples II and III set forth actual operating data accumulated in the use of our novel process.

#### EXAMPLE I

Mixtures of clay and coke in proportions sufficient to supply carbon somewhat in excess of the quantity theoretically required for reducing the oxides present were prepared. These mixtures were charged into a small, laboratory-type electric furnace and were heated to approximately 2000° C. Contrary to expectations, electrode consumption was very high under these conditions and other unfavorable results were obtained. Tapping was difficult and the alloy production rate was low, with a consequent increase in the amount of electrical energy required per pound of alloy produced. Other mixtures were then prepared in which the coke content of the charge was reduced to about 90 per cent of the theoretical carbon requirement. These were charged into the same small furnace and smelted by heating to approximately 2000° C. Steady state operation could not be obtained.

#### EXAMPLE II

Large-scale tests were made in a single phase 600 kw. furnace having a single movable electrode and a conducting hearth which served as the opposite electrode. The furnace was lined with firebrick in the upper portion, carbon blocks in the lower portion and the hearth was composed of carbon blocks 20 inches thick resting on the steel contact plate. The inside dimensions of the crucible were: depth, 3½ feet, diameter at the top, 4½ feet, diameter at hearth, 3¾ feet. A tapping hole 4 inches in diameter extended through a zircon block embedded in the furnace lining at approximately the level of the hearth. Automatic means were used to control the depth of the electrode in the furnace in order to maintain uniform current. In a part of the work, a graphite electrode 12 inches in diameter and 60 inches long was used. In further work, an electrode, formed from amorphous carbon, 17 inches in diameter and 60 inches long was used. Water-cooled electrode holders were used.

The clay used in the tests was calcined in a rotary kiln before charging to the electric furnace. The calcined clay ranged in size up to 2-inch lumps and had the following average chemical composition:

| Al <sub>2</sub> O <sub>3</sub> | SiO <sub>2</sub> | Fe <sub>2</sub> O <sub>3</sub> | TiO <sub>2</sub> | Ignition Loss |
|--------------------------------|------------------|--------------------------------|------------------|---------------|
| Per cent                       | Per cent         | Per cent                       | Per cent         | Per cent      |
| 44.5                           | 50.7             | 0.9                            | 2.8              | 1.0           |

Both byproduct coke and beehive coke in various sizes were used as the reducing agent. The quantity of carbon theoretically required to reduce the furnace charge was calculated as the amount necessary to reduce the oxides of aluminum, silicon, iron and titanium in the clay and in the coke ash in accordance with the equations:



15 Coke was added to the furnace charge in quantities sufficient to provide some 73.5 per cent of the total carbon theoretically required. The calculated amount of coke was mixed with the calcined clay and the mixture added periodically to the furnace around the electrode. The metal 20 was tapped from the furnace at regular intervals, usually about two to two and one-half hours while the furnace was maintained at a temperature of the order of 2000° C. The electrode periphery resistance R was varied and the results 25 shown in the graph in Figure 2 were obtained. The minimum consumption of graphite electrodes was obtained when R was 0.15 ohm-inch. These tests were carried out with 12-inch graphite electrodes.

Other tests were made with 17-inch amorphous carbon electrodes since this type of electrode is used in most commercial ferroalloy operations because of lower cost. Because of the lower current-carrying capacity of carbon electrodes, however, the optimum value of the electrode periphery resistance R was considerably different from that which had been determined when operating with graphite electrodes. The results 30 of a series of four tests in which the resistance was varied while the carbon content of the charge was held constant showed that the best results are obtainable when the electrode periphery resistance R is maintained in the range from 0.30 to 0.36 ohm-inch, with an optimum at 0.33 ohm-inch.

#### EXAMPLE III

The same furnace described in Example II was 50 operated for a period of nine days using graphite electrodes. The operating conditions and results are shown as follows:

##### Operating conditions

|                     |                                              |        |
|---------------------|----------------------------------------------|--------|
| 55                  | Length of period, hr.                        | 216    |
|                     | Total time of operation, hr.                 | 209    |
|                     | Operating time, per cent                     | 96.8   |
| Charge proportions: |                                              |        |
| 60                  | Clay, lb.                                    | 1,000  |
|                     | Coke, lb.                                    | 291    |
|                     | Coke carbon, lb.                             | 275    |
|                     | Carbon in charge, per cent of theoretical    | 73.5   |
| 65                  | Secondary voltage                            | 47     |
|                     | Electrode voltage                            | 44     |
|                     | Current, amp.                                | 11,000 |
|                     | Electrode current density, amp. per sq. in.  | 97     |
|                     | Average k. v. a.                             | 517    |
|                     | Average kw.                                  | 480    |
| 70                  | Power factor                                 | 0.93   |
|                     | Electrode voltage-current ratio (resistance) | 0.004  |
|                     | Electrode periphery resistance,              |        |
| 75                  | $\frac{E}{I} \pi D$ ohm-in.                  | 0.15   |

## Operating results

|                                                |      |
|------------------------------------------------|------|
| Charge consumption:                            |      |
| Clay, lb. per hr.                              | 207  |
| Coke, lb. per hr.                              | 60   |
| Clay, lb. per ton of alloy                     | 4954 |
| Coke, lb. per ton of alloy                     | 1444 |
| Coke carbon, lb. per ton of alloy              | 1364 |
| Alloy production rate, lb. per hr.             | 83   |
| Power consumption, kw.-hr. per lb. of alloy    | 5.7  |
| Electrode consumption, lb. per hr.             | 11.4 |
| Electrode consumption, lb. per ton of alloy    | 274  |
| Total carbon consumed, per cent of theoretical | 88   |
| Composition of alloy:                          | 15   |
| Al, per cent                                   | 51.8 |
| Si, per cent                                   | 38.7 |
| Fe, per cent                                   | 4.9  |
| Ti, per cent                                   | 4.6  |
| Alloy recovery, lb. per ton of clay            | 806  |
| Alloy recovery, per cent                       | 81   |
| Aluminum recovery, per cent                    | 89   |
| Silicon recovery, per cent                     | 65   |

(Values involving the weight of the alloy were calculated from the total weight of metal tapped minus the weight of tapping bars consumed. Values involving power consumption include only the power consumed at the furnace electrode. Power consumed in tapping amounted to from 2 to 5 per cent of the total.)

## EXAMPLE IV

The same furnace used in Example III was equipped with electrodes formed from amorphous carbon and was operated for a 5-day period. The operating conditions and results were as follows:

## Operating conditions

|                                              |        |
|----------------------------------------------|--------|
| Length of period, hr.                        | 120    |
| Total time of operation, hr.                 | 118    |
| Operating time, per cent                     | 98.3   |
| Charge proportions:                          |        |
| Clay, lb.                                    | 1,000  |
| Coke, lb.                                    | 325    |
| Coke carbon, lb.                             | 271    |
| Carbon in charge, per cent of theoretical    | 71.3   |
| Secondary voltage                            | 65     |
| Electrode voltage                            | 61     |
| Current, amp.                                | 9,980  |
| Electrode current density, amp. per sq. in.  | 44     |
| Average k. v. a.                             | 649    |
| Average kw.                                  | 612    |
| Power factor                                 | 0.94   |
| Electrode voltage-current ratio (resistance) | 0.0061 |
| Electrode periphery resistance,              |        |

$$\frac{E}{I} \pi D \text{ ohm-inch} \quad 0.33$$

## Operating results

|                                                |       |
|------------------------------------------------|-------|
| Charge consumption:                            |       |
| Clay, lb. per hr.                              | 258   |
| Coke, lb. per hr.                              | 84    |
| Clay, lb. per ton of alloy                     | 5,333 |
| Coke, lb. per ton of alloy                     | 1,733 |
| Coke carbon, lb. per ton of alloy              | 1,447 |
| Alloy production rate, lb. per hr.             | 97    |
| Power consumption, kw.-hr. per lb. of alloy    | 6.3   |
| Electrode consumption, lb. per hr.             | 13.8  |
| Electrode consumption, lb. per ton of alloy    | 285   |
| Total carbon consumed, per cent of theoretical | 85.7  |

|                                     |      |
|-------------------------------------|------|
| Composition of alloy                |      |
| Al, per cent                        | 46.0 |
| Si, per cent                        | 43.8 |
| Fe, per cent                        | 4.3  |
| Ti, per cent                        | 5.9  |
| Alloy recovery, lb. per ton of clay | 750  |
| Alloy recovery, per cent            | 75   |
| Aluminum recovery, per cent         | 71   |
| Silicon recovery, per cent          | 67   |

10 (Values involving the weight of alloy were calculated from the total weight of the metal tapped minus the weight of the tapping bars consumed. Values involving power consumption include total power consumed at the furnace electrode and at the tapping electrode. Power consumed at the tapping electrode amounted to about 2 per cent of the total.)

15 By use of our novel ratio of carbon to oxides present in the charge, we have obtained lower electrode consumption than has been known in the art of aluminum-silicon alloy production.

20 Use of our novel and advantageous range of values for the electrode periphery resistance R in combination with our novel ratio of carbon to oxides gives a minimum electrode consumption, lowers the power required per ton of alloy produced and gives steady state operation of the furnace. While we do not know the exact causes of these advantageous results, it seems probable that when amounts of carbon approaching the stoichiometric proportion are present in the 25 furnace charge there is a tendency toward the formation of difficultly fusible carbides of silicon and aluminum and that the accumulation of unfused material in the bottom of the furnace causes the electrodes to rise higher and higher 30 as operation continues, with the result that the hot portion of the electrode is forced out of the charge and exposed to air oxidation, and eventually a furnace shut-down to clean out the unfused material becomes necessary. The use of 35 lower resistance to bring the electrode back down is not effective since it does not prevent the accumulation of the unfused material. We have found that the formation of this material does not occur when there is a deficiency of coke present. The limit to which the carbon content can be reduced is the point at which the formation of a slag of unreduced alumina occurs.

Having described our invention and explained its operation, we claim:

40 1. A process for the production of an aluminum-silicon alloy which comprises preparing a charge containing oxides of aluminum and silicon in admixture with carbon as reducing agent; controlling the quantity of such carbon admixed with other materials in preparing said charge so that the ratio of such carbon to total metal oxides present in the charge is in the range from 67 to 85 per cent of the carbon theoretically required for reducing said total oxides; smelting 45 the prepared charge in an electric furnace provided with at least one carbon electrode; maintaining the carbon electrode periphery resistance R in the range from 0.14 to 0.45 ohm-inches during such smelting; and withdrawing aluminum-silicon alloy from the furnace.

50 2. A process for the production of an aluminum-silicon alloy which comprises preparing a charge containing oxides of aluminum and silicon in admixture with carbon as reducing agent; controlling the quantity of such carbon admixed with other materials in preparing said charge so that the ratio of such carbon to total oxides present in the charge is in the range from 60 67 to 75 per cent of the carbon theoretically required for reducing said total oxides; smelting 65

the prepared charge in an electric furnace provided with at least one carbon electrode; maintaining the carbon electrode periphery resistance  $R$  in the range from 0.14 to 0.45 ohm-inches during such smelting; and withdrawing aluminum-silicon alloy from the furnace.

3. A process for the production of an aluminum-silicon alloy which comprises preparing a charge containing oxides of aluminum and silicon in admixture with carbon as reducing agent; controlling the quantity of such carbon admixed with other materials in preparing said charge so that the ratio of such carbon to total oxides present in the charge is in the range from 67 to 85 per cent of the carbon theoretically required for reducing said total oxides; smelting the prepared charge in an electric furnace provided with at least one graphite electrode; maintaining the carbon electrode periphery resistance  $R$  in the range from 0.14 to 0.16 ohm-inches during such smelting; and withdrawing aluminum-silicon alloy from the furnace.

4. A process for the production of an aluminum-silicon alloy which comprises preparing a charge containing oxides of aluminum and silicon in admixture with carbon as reducing agent; controlling the quantity of such carbon admixed with other materials in preparing said charge so that the ratio of such carbon to total oxides present in the charge is in the range from 70 to 75 per cent of the carbon theoretically required for reducing said total oxides; smelting the prepared charge in an electric furnace provided with at least one graphite electrode; maintaining the carbon electrode periphery resistance  $R$  in the range from 0.14 to 0.16 ohm-inches during such smelting; and withdrawing aluminum-silicon alloy from the furnace.

5. A process for the production of an aluminum-silicon alloy which comprises preparing a charge containing oxides of aluminum and silicon in admixture with carbon as reducing agent; controlling the quantity of such carbon admixed with other materials in preparing said charge so that the ratio of such carbon to total oxides present in the charge is in the range from 67 to 85 per cent of the carbon theoretically required for reducing said total oxides; smelting the prepared charge in an electric furnace provided with at least one amorphous carbon electrode; maintaining the carbon electrode periphery resistance  $R$  in the range from 0.30 to 0.45 ohm-inches during such smelting; and withdrawing aluminum-silicon alloy from the furnace.

6. A process for the production of an aluminum-silicon alloy which comprises preparing a charge containing oxides of aluminum and silicon in admixture with carbon as reducing agent; controlling the quantity of such carbon admixed with other materials in preparing said charge so that the ratio of such carbon to total oxides present in the charge is in the range from 70 to 75 per cent of the carbon theoretically required for reducing said total oxides; smelting the prepared charge in an electric furnace provided with at least one amorphous carbon electrode; maintaining the carbon electrode periphery resistance  $R$  in the range from 0.30 to 0.45 ohm-inches during such smelting; and withdrawing aluminum-silicon alloy from the furnace.

7. A process for the production of an aluminum-silicon alloy which comprises preparing a charge containing clay in admixture with carbon as reducing agent; controlling the quantity of

such carbon admixed with other materials in preparing said charge so that the ratio of such carbon to total oxides present in the charge is in the range from 67 to 85 per cent of the carbon theoretically required for reducing said total oxides; smelting the prepared charge in an electric furnace provided with at least one graphite electrode; maintaining the carbon electrode periphery resistance  $R$  in the range from 0.14 to 0.16 ohm-inches during such smelting; and withdrawing aluminum-silicon alloy from the furnace.

8. A process for the production of an aluminum-silicon alloy which comprises preparing a charge containing clay in admixture with carbon as reducing agent; controlling the quantity of such carbon admixed with other materials in preparing said charge so that the ratio of such carbon to total oxides present in the charge is in the range from 70 to 75 per cent of the carbon theoretically required for reducing said total oxides; smelting the prepared charge in an electric furnace provided with at least one graphite electrode; maintaining the carbon electrode periphery resistance  $R$  in the range from 0.14 to 0.16 ohm-inches during such smelting; and withdrawing aluminum-silicon alloy from the furnace.

9. A process for the production of an aluminum-silicon alloy which comprises preparing a charge containing clay in admixture with carbon as reducing agent; controlling the quantity of such carbon admixed with other materials in preparing said charge so that the ratio of such carbon to total oxides present in the charge is in the range from 67 to 85 per cent of the carbon theoretically required for reducing said total oxides; smelting the prepared charge in an electric furnace provided with at least one amorphous carbon electrode; maintaining the carbon electrode periphery resistance  $R$  in the range from 0.30 to 0.45 ohm-inches during such smelting; and withdrawing aluminum-silicon alloy from the furnace.

10. A process for the production of an aluminum-silicon alloy which comprises preparing a charge containing clay in admixture with carbon as reducing agent; controlling the quantity of such carbon admixed with other materials in preparing said charge so that the ratio of such carbon to total oxides present in the charge is in the range from 70 to 75 per cent of the carbon theoretically required for reducing said total oxides; smelting the prepared charge in an electric furnace provided with at least one amorphous carbon electrode; maintaining the carbon electrode periphery resistance  $R$  in the range from 0.30 to 0.45 ohm-inches during such smelting; and withdrawing aluminum-silicon alloy from the furnace.

11. In the production of an aluminum-silicon alloy where a charge comprising oxides of aluminum and silicon in admixture with carbon as reducing agent is introduced into an electric furnace provided with at least one carbon electrode and is smelted therein, that improvement which comprises reducing consumption of carbon electrode by controlling the quantity of carbon admixed with said oxides so that the ratio of carbon to total oxides contained in the resulting charge is in the range from 67 to 85 per cent of the ratio theoretically required for reducing said total oxides.

12. The process of claim 11 wherein the ratio of carbon to total oxides in the charge is con-

**11**

trolled in the range from 70 to 75 per cent of the amount theoretically required for reducing said total oxides.

MARCUS M. STRIPLIN, JR.  
WILLIAM M. KELLY.

**REFERENCES CITED**

The following references are of record in the file of this patent:

**12****UNITED STATES PATENTS**

Number Name Date  
1,594,362 Frary ----- Aug. 3, 1926

**FOREIGN PATENTS**

Number Country Date  
5 302,692 Great Britain ----- Dec. 20, 1927